

# UNITED STATES PATENT OFFICE.

KARL KREKELER AND EDUARD MARTZ, OF ELBERFELD, GERMANY,  
ASSIGNORS TO THE FARBENFABRIKEN OF ELBERFELD COMPANY,  
OF NEW YORK, N. Y.

## BROWN TRISAZO DYE.

### SPECIFICATION forming part of Letters Patent No. 602,858, dated April 26, 1898.

Application filed November 23, 1897. Serial No. 659,582. (Specimens.) Patented in Germany September 15, 1891, No. 65,262; in England December 28, 1891, No. 22,641; in France April 28, 1892, No. 221,233; in Italy June 30, 1892, XXVI, 32,191, and LXIII, 186, and in Austria-Hungary October 3, 1892, No. 1,242 and No. 16,870.

To all whom it may concern:

Be it known that we, KARL KREKELER and EDUARD MÁRTZ, doctors of philosophy, chemists, of Elberfeld, Germany, (assignors to the 5 FARBENFABRIKEN OF ELBERFELD COMPANY, of New York,) have invented a new and useful Improvement in the Manufacture of Brown Trisazo Dye, (for which the Farbenfabriken, vormals Fr. Bayer & Co., of Elberfeld, Germany, has already obtained Letters Patent 10 in Germany, No. 65,262, dated September 15, 1891; in England, No. 22,641, dated December 28, 1891; in France, No. 221,233, dated April 28, 1892; in Italy, Reg. Gen., Vol. XXVI, 15 No. 32,191, Reg. Att., Vol. LXIII, No. 186, dated June 30, 1892, and in Austria-Hungary, No. 1,242 and No. 16,870, dated October 3, 1892;) and we hereby declare the following to 20 be a clear and exact description of our invention.

Our invention relates to the production of a new class of trisazo dyestuffs by diazotizing tetrazo bodies of the general formula



in which formula P represents a radical of the benzidin series, such as diphenyl, ditolyl, 30 diphenyl ether, or the like; R, the radical of an orthoöxycarbonic acid of the benzene series, such as salicylic acid or cresotinic acid; C, the radical of the so-called "Clève's alpha-naphthylamin-beta-sulfonic acid" (1.6 or 1.7) 35 and combining the diazo body thus obtained with one molecule of an orthoöxycarbonic acid, such as salicylic acid or cresotinic acid. The dyestuffs thus obtained have the general formula



(P, R, and C meaning in this formula the 45 above-defined radicals.) They represent dark powders which dissolve in water with a color varying from yellowish brown to brown and

dye cotton from yellowish-brown to brown shades, which, by a treatment with a solution of bichromate of soda or of an analogous 50 chromium salt, with or without the presence of copper salts, become more reddish brown and faster to washing and against the action of light. The new coloring-matters are also capable of dyeing wool in acid-baths. The 55 shades thus obtained are similar to those produced on cotton.

In carrying out our new process practically we can proceed as follows: 18.4 kilos, by weight, of benzidin are diazotized in the usual 60 manner by means of fourteen kilos, by weight, of sodium nitrite. To the icy-cold diazo solution an icy-cold solution of fourteen kilos, by weight, of salicylic acid and seventy kilos, by weight, of sodium carbonate ( $\text{Na}_2\text{CO}_3$ ) in 65 four hundred liters of water is added with stirring. When the formation of the intermediate product is finished, a cold solution prepared by dissolving 24.5 kilos, by weight, of the sodium salt of alpha-naphthylamin-beta-monosulfo-acid (1.6) in three hundred 70 liters of water is added. After about a three hours' stirring the formation of the intermediate dyestuff is complete. The mixture is subsequently acidulated by means of hydrochloric acid and filtered. The dyestuff acid thus obtained is dissolved in fifteen hundred 75 liters of a 2.5-per-cent. soda-lye, then quickly mixed with a solution of eight kilos, by weight, of sodium nitrite, five hundred kilos, by weight, of ice, and one hundred and fifty kilos, by weight, of hydrochloric acid, (20° Baumé.) This mixture is stirred for about 80 twelve hours, and then the resulting insoluble diazo compound is filtered and pressed. 85 Subsequently it is mixed with ice and water to a thin paste, which is slowly stirred into an icy-cold concentrated solution of fourteen kilos, by weight, of salicylic acid and one hundred and forty kilos, by weight, of sodium 90 carbonate. After stirring for twelve hours the mixture is heated to about 70° centigrade. The dyestuff thus complete is salted out in the usual manner. Then it is filtered off,

pressed, dried, and pulverized. It is the sodium salt of an acid having the formula:



and represents a dark-brown powder, soluble in water with a yellowish-brown color and in concentrated sulfuric acid with a blue color.

15 From this solution a dark-brown flaky precipitate is obtained on the addition of a sufficient quantity of ice.

The new coloring-matter dyes unmordanted cotton yellowish-brown shades, which when treated with a solution of a chromium salt, with or without the presence of salts of copper, become more reddish brown and faster to washing and against the action of light.

On unmordanted wool the coloring-matter 25 produces in acid-baths yellowish-brown shades, which on a treatment with chromium salts become fast against milling.

Having now described our invention and in what manner the same is to be performed, what we claim as new, and desire to secure by Letters Patent, is—

1. The process for producing new trisazo dyestuffs by combining the diazo derivatives of the disazo compounds hereinbefore defined, such as the combination of one molecule of tetrazodiphenyl with one molecule of salicylic acid and one molecule of Clève's naphthylaminsulfo-acid, having the general formula

4°  $\text{P} \begin{cases} \text{N}=\text{N}-\text{ortho}\text{oxy}\text{carbonic acid} \\ \text{N}=\text{N}-\text{Clève's naphthylamininsulfo-acid} \end{cases}$

45 with one molecule of an ortho&oxycarbonic acid of the benzene series substantially as hereinbefore described.

2. The process for producing a new trisazo dyestuff by combining the diazo derivative of the body having the formula

50 Benzidin (tetrazotized)  Salicylic acid  
Clève's naphthylaminosulfo-acid  
with one molecule of salicylic acid substituted

55 3. As new articles of manufacture the new trisazo dyestuffs obtainable from the diazo

exists by means obtainable from the author.

derivatives of the disazo compounds, such as the combination of one molecule of tetrazodiphenyl with one molecule of salicylic acid and one molecule of Clève's naphthylamin-<sup>60</sup> sulfo-acid, having the general formula:



with one molecule of an orthoöxycarbonic acid of the benzene series, being dark powders, soluble in water with a color varying from yellowish brown to brown, dyeing unmordanted cotton from yellowish-brown to 70 brown shades which when treated with solutions of chromium and copper salts become more reddish brown and faster to washing and against the action of light, capable of dyeing wool in acid-baths shades similar to those 75 produced on cotton substantially as described.

4. As a new article of manufacture the specific dyestuff obtainable from the diazo derivative of the body, having the formula: 80



with one molecule of salicylic acid being an alkaline salt of an acid having the formula 85



representing in the form of the sodium salt a dark-brown powder, soluble in water with a yellowish-brown color, in concentrated sulfuric acid with a blue color from which solution a dark-brown flaky precipitate is obtained on the addition of a sufficient quantity of ice, dyeing unmordanted cotton yellowish-brown shades which when treated with solutions of chromium and copper salts become more reddish brown and faster to washing and against the action of light, yielding on wool in acid-baths yellowish-brown shades which on a treatment with chromium salts become fast against milling substantially as described. 90 95 100

In testimony whereof we have signed our names in the presence of two subscribing witnesses. 105

KARL KREKELER.  
EDUARD MARTZ.

**Witnesses:**

R. E. JAHN,  
OTTO KÖNIG.